

March 2, 1954

J. J. BROPHY

2,670,483

STIFFENING PORTION OF SHOES

Filed Oct. 5, 1951



*Inventor*

*John J. Brophy*

*By his Attorney*

*Wm. C. Clegg*

## UNITED STATES PATENT OFFICE

2,670,483

## STIFFENING PORTION OF SHOES

John J. Brophy, Salem, Mass., assignor to United Shoe Machinery Corporation, Flemington, N. J., a corporation of New Jersey

Application October 5, 1951, Serial No. 249,991

6 Claims. (Cl. 12—146)

1

This invention relates to a method of stiffening selected portions of shoes, and more particularly to a method of stiffening such portions by so treating stiffener material incorporated in limp condition into the shoe materials as to convert the stiffener material to a stiffer, but resilient condition.

In the manufacture of shoes, it is frequently desirable to provide a stiffener member within the shoe, for example, at the shank, toe or heel portions. One method of stiffening toe or heel portions has been to include between the layers of upper materials a preformed blank of fiberboard. An advantageous method, disclosed, for example, in United States Letters Patent No. 2,406,738 granted September 3, 1946, and United States Letters Patent No. 2,539,608 granted January 30, 1951 both in the name of John J. Brophy, comprises the steps of incorporating into the upper materials, at any convenient time prior to lasting, a limp blank which is convertible to a stiffer, but resilient condition and converting the blank to such a condition by subjecting it to the heating effect of an alternating electric field following the lasting step. This method has provided many shoemaking advantages, for example in added convenience of handling the upper materials prior to lasting and in enhanced quality of the product resulting in part from the better lasting obtainable therewith. However, normally moist leather is susceptible to damage by heat and has a dielectric loss in the same order of magnitude as many of the proposed stiffener blanks. Owing to these physical and electrical characteristics of leather, the electric field must presently be applied within fairly critical power-time limits in order properly to convert the stiffener blank without damage to the shoe. Further, whatever form of heat is employed, a large portion of the treatment cycle is occupied in bringing the stiffener material up to converting temperature and hence the treatment is not immediately effective to promote conversion.

Accordingly an object of the invention is the provision of an improved method of providing a stiffening portion in a shoe which will retain the advantages of the above dielectric process while overcoming attendant difficulties.

Another object of the invention is the provision of a method of stiffening a selected portion of a shoe by treating, for conversion to a stiffer, but resilient mass, limp stiffener material incorporated into the shoe materials in the selected area, in which method the treatment may be performed very rapidly without damage to the shoe parts.

2

In one aspect, the invention comprises a method wherein stiffener material is incorporated in limp condition into the shoe materials in the area to be stiffened, and the stiffener material is converted to a stiffer, but resilient condition by subjecting it to "materialistic radiation" such as high speed electrons. "Materialistic radiation" as used herein, includes "material radiation" in the sense used in Pollard and Davidson, Applied Nuclear Physics, John Wiley and Sons 1942, pp. 10 et seq., and also includes X-rays and gamma rays. Such subjection in accordance with the present invention usually involves projecting such radiation through intervening shoe material, for example, through an outer layer of upper leather, but such delicate and heat-sensitive materials are unharmed during the short time required for activation.

These and other features and advantages of 20 the invention will best be understood from the following description taken in connection with the accompanying drawings in which:

Fig. 1 is a perspective view illustrating the activation of stiffener material within the toe 25 portion of a lasted shoe; and

Fig. 2 is an enlarged section through the toe of said shoe.

Referring to Figs. 1 and 2, the shoe 10 has incorporated in its upper at the toe in limp form, stiffener material, preferably in the form of a limp stiffener blank 12. Various methods of preparing such blanks are disclosed in the patents referred to above. Typically, a blank may be cut from a sheet comprising a porous base which has been first impregnated with a solution of a stiffener composition and then dried.

The conversion step is illustrated diagrammatically in Fig. 1. The shoe is prepared by incorporating a limp stiffener blank in the upper materials in the portion to be stiffened and lasting the upper over an insole. If the shoe upper materials include a lining, this may be adhesively secured to the stiffener blank at a convenient time prior to lasting, for example, by pressing a lining and blank together momentarily against a heated surface to apply a little heat through the lining. The toe of the lasted shoe 10 is shown subjected to a beam 14 of high-speed electrons from a source 16. Apparatus of various types for providing a beam of such electrons is commercially available, and being well-known, a particular source will not be described here. Such a beam is considered herein as comprising electron radiation.

55 The electron speed should be high enough so that electrons penetrate the outer layers of the

upper or any other intervening material and traverse the stiffener material. I have found voltages from about 0.4 to 3 million volts to be very satisfactory for treating stiffening material beneath leather, but higher or lower voltages may be used as circumstances warrant.

If it is desired to treat the blank at minimum voltage, the shoe may be rocked or tilted during subjection to the beam so that the sides and feather edge areas 18 are presented to the beam. I have found, however, that at 3 million volts, these areas are completely converted by a beam directed toward the top of the toe, presumably by secondary electrons produced by ionization of the air adjacent to these areas.

Compositions suitable for preparing a stiffener blank which is initially limp but convertible to a resilient condition in accordance with the present invention may comprise, for example, a polymerizable compound, preferably, a polyunsaturated ester of the type disclosed in United States Letters Patent No. 2,155,590 granted April 25, 1939, on an application filed in the name of Benjamin S. Garvey. Commercially available materials containing esters of this type include various so-called unsaturated polyester resins: Plaskon 920/2 made by Libby-Owens-Ford Glass Company, Toledo, Ohio; Paraplex P-43 and P-13 made by Rohm and Haas, Philadelphia, Pennsylvania; Laminac 4-201 and 4-128 made by American Cyanamid and Chemical Corporation, Plastics Division, New York, New York; Vibrin 120 and 1305 made by the Naugatuck Chemical Company, Naugatuck, Connecticut; and Castolite made by the Castolite Company, Woodstock, Illinois.

To the polymerizable compound we prefer to add a plasticizable solid, such as an alkyd resin or a vinyl chloride vinyl acetate copolymer, to enhance the resilience of the converted blank.

The following examples are given for purposes of illustration to aid in understanding the invention and it is to be understood that the invention is not limited to the specific materials or operating conditions disclosed.

#### Example I

A shoe was prepared by incorporating into the upper in the toe region a stiffener blank comprising a single nap cotton flannel impregnated to comprise 80 per cent solids of the following stiffener composition:

|                                                | Parts by weight |
|------------------------------------------------|-----------------|
| Vinylite VYHH                                  | 30.5            |
| Polyethylene glycol 200 dimethacrylate monomer | 15.25           |
| Benzoyl peroxide                               | 0.15            |
| Tricresyl phosphate                            | 0.15            |
| Acetone                                        | 57              |
| p-Phenyl phenol (inhibitor)                    | 0.076           |

Vinylite VYHH is a copolymer of vinyl chloride and vinyl acetate comprising about 15 per cent vinyl acetate and is produced by Carbide and Carbon Chemicals Corporation of New York. The polyethylene monomer is an ester of methacrylic acid and polyethylene glycol 200 obtained from Carbide and Carbon Chemicals Corporation of New York. The lasted shoe was placed on a conveyor belt with the upper up and thereby moved at 0.4 inch per second beneath the window of an electron accelerator of the type disclosed in United States Letters Patent No. 1,991,236 issued February 12, 1935, in the name of Robert J. Van de Graaff for an exposure of about 10 seconds at a distance of 40 centimeters from the window. 75

The current of the beam was 100 microamperes, corresponding to a density of about 1.46 microamperes per square centimeter, and the voltage was 3 million volts.

5 The box toe was exceedingly well converted in a very uniform manner over its entire surface even in the feather line region which was not in the direct path of the beam and with no apparent deleterious effect on either the upper leather or any other shoe component.

#### Example II

The procedure of Example I was carried out with a stiffener blank impregnated with a stiffener composition which was similar to that of Example I, but in which the benzoyl peroxide was omitted. After subjection to the beam, the toe was well and uniformly converted.

#### Example III

15 A quantity of Vibrin 1305 which has a wax-like consistency at room temperature, was warmed to 50-60° C. at which temperature the viscosity was reduced sufficiently to impregnate a double nap flannel. The impregnated flannel was allowed to cool, and a box toe blank was cut from it and incorporated in the upper of a shoe which was then lasted.

20 The blank was then treated as described in Example I, producing a very satisfactory box toe.

#### Example IV

25 Three parts by weight of Atlac 382, an unsaturated alkyd resin made by the Atlas Powder Company of Wilmington, Delaware, and one part of diallyl phthalate were dissolved in four parts of benzene. A double nap flannel was impregnated with this solution and dried. A box toe blank cut from this impregnated flannel was incorporated in the toe of a lasted shoe and the blank treated as described in Example I, producing a very satisfactory shoe.

#### Example V

30 A limp box toe blank made as in Example I was subjected to the beam from the electron accelerator at 1.5 million volts for a period of  $2 \pm 1$  seconds. The blank was thereafter found to be very resilient.

#### Example VI

35 A limp box toe blank was prepared as in Example II. After treatment at 1.5 million volts for  $2 \pm 1$  seconds, it was converted to a resilient condition.

40 While I have disclosed the use of an electron beam for treating the convertible stiffener material, it will be understood that the stiffener material may be subjected, for treatment purposes, to other forms of materialistic radiation in the nature of X-rays, gamma rays, protons, deuterons, neutrons, ions and alpha particles.

Having thus described my invention, what I claim as new and desire to secure by Letters Patent of the United States is:

45 1. The method of producing a stiffening portion in a shoe comprising the steps of incorporating in a selected part of a shoe, in limp form, stiffener material convertible through polymerization to a stiffer, but resilient resinous condition, and subjecting the stiffener material to materialistic radiation to effect such conversion.

50 2. The method of claim 1 in which the radiation is material radiation.

3. The method of claim 1 in which the radiation is electron radiation.

4. The method of producing a stiffening portion in a shoe comprising the steps of incorporating in a selected portion of a shoe, in limp form, stiffener material comprising an unsaturated ester and subjecting the stiffener material to materialistic radiation to convert it to a stiffer, but resilient condition.

5. The method of claim 4 in which the radiation is material radiation.

6. The method of claim 4 in which the radiation is electron radiation.

## References Cited in the file of this patent

## UNITED STATES PATENTS

| Number    | Name   | Date          |
|-----------|--------|---------------|
| 1,818,073 | Long   | Aug. 11, 1931 |
| 1,906,402 | Newton | May 2, 1933   |
| 2,155,590 | Garvey | Apr. 25, 1939 |
| 2,429,217 | Brasch | Oct. 21, 1947 |
| 2,539,608 | Brophy | Jan. 30, 1951 |

JOHN J. BROPHY.